# EUROPEAN PATENT SPECIFICATION

(11) **EP 3 861 089 B1**
(45) Date of publication and mention of the grant of the patent: **25.12.2024**
(21) Application number: 19783721.4
(22) Date of filing: 02.10.2019
(51) Int. Cl.: C10L 1/14, C10L 10/10, C10L 10/12, C10M 127/04, C10M 129/16, C10M 133/38, C10L 1/16, C10L 1/185, C10L 1/232, C10L 1/233

(54) **HYDRIDE DONORS AS AN ADDITIVE FOR REDUCING LOW SPEED PRE-IGNITION EVENTS**
HYDRIDDONOREN ALS ADDITIV ZUR REDUZIERUNG VON VORZÜNDUNGSEREIGNISSEN BEI NIEDRIGER GESCHWINDIGKEIT
DONNEURS D'HYDRURE UTILISÉS EN TANT QU'ADDITIF POUR RÉDUIRE DES ÉVÉNEMENTS DE PRÉ-ALLUMAGE À FAIBLE VITESSE

(30) Priority: 04.10.2018 US 201862741229 P
(43) Date of publication of application: 11.08.2021
(73) Proprietor: Chevron Oronite Company LLC, San Ramon, CA 94583 (US); Chevron U.S.A. Inc., San Ramon, CA 94583 (US)
(72) Inventor: CHERPECK, Richard Eugene, San Ramon, California 94583-0806 (US); ELLIOTT, Ian G., San Ramon, California 94583-0806 (US); GUNAWAN, Theresa Liang, San Ramon, California 94583-0806 (US); MARIA, Amir Gamal, San Ramon, California 94583-0806 (US)
(74) Representative: Haseltine Lake Kempner LLP
(86) International application number: PCT/IB2019/058397
(87) International publication number: WO 2020/070672

(56) References cited:
- WO-A1-2017/081116
- WO-A2-2018/172911
- DE-A1- 102016 116 348
- US-A- 2 754 216
- US-A- 4 457 763
- US-A- 6 156 081
- US-A1- 2012 129 744
- US-A1- 2016 230 115

## Description

### TECHNICAL FIELD

This disclosure relates to fuel and lubricant compositions and methods of using the compositions to reduce low speed pre-ignition activity in combustion engines. The compositions include organic hydride donors as fuel or lubricant additives.

### BACKGROUND

Pre-ignition in combustion engines is an undesirable event in which undesired ignition of an air-fuel mixture occurs prior to a desired ignition (e.g., via spark plug) of the air-fuel mixture. Pre-ignition can be a problem during high load engine operation since heat from operation of the engine may heat a part of a combustion chamber to a sufficient temperature to ignite the air-fuel mixture upon contact.

In recent years, engine manufacturers have developed smaller engines that provide higher power densities and excellent performance while reducing frictional and pumping losses. This performance improvement is accomplished by increasing boost pressures with use of turbochargers or mechanical superchargers, and by down-speeding the engine using higher transmission gear ratios allowed by higher torque generation at lower engine speeds. A downside is that these engines often operate in low speed and high load driving conditions, making the engines more susceptible to a pre-ignition phenomena known as stochastic pre-ignition or low speed pre-ignition (LSPI). In worst case scenarios, extremely high cylinder peak pressure builds up and leads to catastrophic engine failure. This susceptibility prevents engine manufacturers from fully optimizing engine torque at lower engine speed in such smaller, high-output engines. US 2016/230115 A1 concerns the reduction / prevention of low-speed pre-ignition events in internal combustion engines by using a lubricant composition comprising a base oil and an ashless antioxidant, i.a., diarylamine compounds. DE 10 2016 116348 A1 discloses the addition of aromatic or aliphatic amines additives to reduce or prevent LSPI events in gasoline fuels.

### SUMMARY

In one aspect, there is provided a fuel composition comprising (1) greater than 50 wt. % of a hydrocarbon fuel boiling in the gasoline or diesel range and (2) a minor amount of one or more of organic hydride-based reductant.

In another aspect, there is provided a method for preventing or reducing low speed pre-ignition events in an internal combustion engine, the method comprising supplying to the engine a fuel composition comprising (1) greater than 50 wt. % of a hydrocarbon fuel boiling in the gasoline or diesel range and (2) a minor amount of one or more of organic hydride-based reductant.

In a further aspect, there is provided a lubricating oil composition comprising (1) greater than 50 wt. % of a base oil and (2) a minor amount of one or more of organic hydride-based reductant.

In yet a further aspect, there is provided a method for preventing or reducing low speed pre-ignition events in a spark-ignited internal combustion engine, the method comprising supplying to the engine a lubricating oil composition comprising (1) greater than 50 wt. % of a base oil and (2) a minor amount of one or more of organic hydride-based reductant.

### DETAILED DESCRIPTION

The present invention is disclosed in and by the appended claims.

### Definitions

In this specification, the following words and expressions, if and when used, have the meanings ascribed below.

The term "boosting" refers to running an engine at higher intake pressures than in naturally aspirated engines. A boosted condition can be reached by use of a turbocharger (driven by exhaust) or by a supercharger (driven by engine). Boosting allows engine manufacturers to use smaller engines that provide higher power densities to provide excellent performance while reducing frictional and pumping losses.

The term "oil soluble" means that for a given additive, the amount needed to provide the desired level of activity or performance can be incorporated by being dissolved, dispersed or suspended in an oil of lubricating viscosity. Usually, this means that at least 0.001% by weight of the additive can be incorporated in a lubricating oil composition. The term "fuel soluble" is an analogous expression for additives dissolved, dispersed or suspended in fuel.

"Gasoline" or "gasoline boiling range components" refers to a composition containing at least predominantly C₄-C₁₂ hydrocarbons. In one embodiment, gasoline or gasoline boiling range components is further defined to refer to a composition containing at least predominantly C₄-C₁₂ hydrocarbons and further having a boiling range of from about 37.8°C (100° F) to about 204°C (400°F). In an alternative embodiment, gasoline or gasoline boiling range components is defined to refer to a composition containing at least predominantly C₄-C₁₂ hydrocarbons, having a boiling range of from about 37.8°C (100° F) to about 204°C (400°F), and further defined to meet ASTM D4814.

The term "diesel" refers to middle distillate fuels containing at least predominantly C₁₀-C₂₅ hydrocarbons. In one embodiment, diesel is further defined to refer to a composition containing at least predominantly C₁₀-C₂₅ hydrocarbons, and further having a boiling range of from about 165.6°C (330°F) to about 371.1°C (700°F). In an alternative embodiment, diesel is as defined above to refer to a composition containing at least predominantly C₁₀-C₂₅ hydrocarbons, having a boiling range of from about 165.6°C (330°F) to about 371.1°C (700°F), and further defined to meet ASTM D975.

The term "alkyl" refers to saturated hydrocarbon groups, which can be linear, branched, cyclic, or a combination of cyclic, linear and/or branched.

A "minor amount" means less than 50 wt. % of a composition, expressed in respect of the stated additive and in respect of the total weight of the composition, reckoned as active ingredient of the additive.

A "reductant" is a reducing agent that donates an electron to another chemical species in a redox reaction. A "hydride-based reductant" donates a hydride (anion of hydrogen) to another chemical species during a redox reaction.

In the context of hydrocarbon-based formulations (particularly lubricants), the term "ash" refers to metallic compounds remaining after hydrocarbons have been calcinated. This ash is mainly derived from chemicals used in certain additives, as well as solids. The term "ashless" refers to formulations or additives that do not generate ash or limit generation of ash. Ashless additives are generally free of metals (including boron), silicon, halogen, or contain these elements in concentrations below typical instrument detection limits.

"Halogen" is a collective term for individual substituents that include, for example, fluorine, chlorine, bromine, iodine, and the like.

An "analog" is a compound having a structure similar to another compound but differing from it in respect to a certain component such as one or more atoms, functional groups, substructures, which are replaced with other atoms, groups, or substructures.

A "homolog" is a compound belonging to a series of compounds that differ from each other by a repeating unit. Alkanes are examples of homologs. For example, ethane and propane are homologs because they differ only in the length of a repeating unit (-CH₂-). A homolog may be considered a specific type of analog.

A "derivative" is a compound that is derived from a similar compound via a chemical reaction (e.g., acid-base reaction, hydrogenation, etc.). In the context of substituent groups, a derivative may be a combination of one or more moiety. For example, a phenol moiety may be considered a derivative of aryl moiety and hydroxyl moiety. A person of ordinary skill in the related art would know the metes and bounds of what is considered a derivative.

An "engine" or a "combustion engine" is a heat engine where the combustion of fuel occurs in a combustion chamber. An "internal combustion engine" is a heat engine where the combustion of fuel occurs in a confined space ("combustion chamber"). A "spark ignition engine" is a heat engine where the combustion is ignited by a spark, usually from a spark plug. This is contrast to a "compression-ignition engine," typically a diesel engine, where the heat generated from compression together with injection of fuel is sufficient to initiate combustion without an external spark.

### Introduction

One possible cause of low speed pre-ignition (LSPI) is auto-ignition of engine oil droplets that enter an engine combustion chamber from a piston crevice under high pressure, during periods when the engine is operating at low speeds and compression stroke time is longest. Factors such as turbocharger use, engine design, engine coatings, piston shape, fuel choice, or engine oil additives may contribute to an increase in LSPI events. Although some engine knocking and pre-ignition problems can be resolved through use of new engine technology or optimization of engine operating conditions, reducing LSPI through new fuel and/or lubricant oil compositions may be the most cost-effective approach.

The present disclosure describes hydrocarbon-based compositions (e.g., fuel, lubricating oil) and methods of use thereof, wherein the hydrocarbon-based compositions prevent LSPI events or reduce LSPI activity during operation of a combustion engine. A suitable hydrocarbon-based composition will feature an organic hydride-based reductant additive in accordance with this disclosure.

### Organic Hydride-Based Reductant

The reductants suitable according to the present invention are as defined in the appended claims.

Provided herein are organic hydride-based reductants that prevent LSPI events or reduce LSPI activity in combustion engines. These organic hydride-based reductants are organic molecules prone to donate hydrides during a hydride transfer step. These reductants are ashless additives and usually contain carbon, hydrogen, nitrogen and/or oxygen atoms. Depending on the application, the organic hydride-based reductant is oil soluble or fuel soluble.

Hydride transfer is a key step in many well-known organic reactions including important biochemical and industrial redox reactions. In these types of reactions, reductants provide a hydride (H⁻) that is transferred to substrates such as carbonyl compounds, carbon dioxide, imines, compounds containing activated C=C bonds and the like. Precise mechanism of hydride transfer is often complex and may vary with temperature, substrate, hydride donor, availability of protons, presence of Lewis acid and the like. In some cases, hydride transfer may proceed by direct transfer of hydride ion from hydride donor to the substrate or may occur in consecutive steps (e.g., transfer of electron to the substrate followed by a hydrogen atom or by a proton and second electron).

Without being limited by theory, it is believed that a suitable hydride donor in accordance with the present invention can lower LSPI activity in a combustion engine by acting against oxidatively unstable chemical species that can initiate LSPI events. This may involve reduction of the oxidative unstable chemical species to a more stable, less reactive reduced species, thus inhibiting LSPI events.

According to one or more embodiments disclosed, the organic hydride-based reductant includes at least one of the following organic hydride donors: dihydropyridine (DHPD), reduced nicotinamide adenine dinucleotide (NADH), methylene tetrahydromethanopterin, acridine, triarylmethane, triamine, aryl benzoimidazoline, dioxolane, diethercyclohexadiene, cycloheptatriene, flavin adenine dinucleotide (FADH₂), hexahydro triazaphenalene, an analog thereof, a homolog thereof, and a derivative thereof.

The following chemical structures of organic hydride-based reductants are provided for illustration. Each reductant or reductant-type is represented by a generalized structure that includes generic R groups (e.g., R₁, R₂, R₃, etc.) in various substitution positions. Each R group may be a component selected from a group of suitable substituents. Varying the combination of the R group substituents can result in a set of related structures, wherein each resulting structure is an analog of the other structures within the set. Desirability of a particular substituent may depend on a number of factors including, but not limited to, organic hydride-based donor's target ability to donate hydrides, stability, solubility in oil or fuel, and the like.

### Dihydropyridine (DHPD)

DHPD or DHPD-type reductant is illustrated by a generalized structure (Formula 1). Referring to Formula 1, R₁, and R₂, are each components independently selected from the following group: H, ester moiety, amide moiety, cyanide moiety, any derivative thereof, and the like. R₃ and R₄ are each components independently selected from the following group: H, alkyl moiety, any derivative thereof, and the like. R₅ is a component selected from the following group: H, alkyl moiety, allyl moiety, aryl moiety, benzyl moiety, alkanol moiety, any derivative thereof, and the like.

According to the invention, the compounds are

### Reduced Nicotinamide Adenine Dinucleotide (NADH)

NADH or NADH-type reductant is illustrated by a generalized structure (Formula 2). Referring to Formula 2, R₁ and R₂ are each components independently selected from the following group: H, ester moiety, amide moiety, cyanide moiety, any derivative thereof, and the like. R₃ and R₄ are each components independently selected from the following group: H, alkyl moiety, any derivative thereof, and the like. R₅ is a component selected from the following group: H, alkyl moiety, allyl moiety, aryl moiety, benzyl moiety, alkanol moiety, any derivative thereof, and the like. R₆ is selected from the following group: H, alkyl moiety, any derivative thereof, and the like. In some embodiments, R₁ and R₄ or R₂ and R₃ may form a cyclic or heterocyclic structure (e.g., Formula 2C and 2E).

According to the invention the compounds are

### Methylene Tetrahydromethanopterin

Methylene tetrahydromethanopterin or methylene tetrahydromethanopterin-type reductant is illustrated by a generalized structure (Formula 3). Referring to Formula 3, R₁, R₂, R₃, and R₄ are each components independently selected from the following group: H, alkyl moiety, allyl moiety, alkanol moiety. R₅ is selected from the following group: H, alkyl moiety, any derivative thereof, and the like.

Suitable analogs of methylene tetrahydromethanopterin include

### Acridine

Acridine or acridine-type reductant is illustrated by a generalized structure (Formula 4). Referring to Formula 4, X is N or O (Formula 4H). When X is N, R₁ is selected from the following group: H, alkyl moiety, allyl moiety, aryl moiety, benzyl moiety, R₂ is selected from the following group: H, alkyl moiety, allyl moiety, aryl moiety, benzyl moiety, alkanol moiety, R₃ and R₄ are each components independently selected from the following group: H, alkyl moiety, aryl moiety, benzyl moiety, amine moiety, alkoxy moiety, heteroatoms, Moreover, R₃ as well as R₄ may independently occupy more than one substitution position within its respective rings. In some embodiments, R₁ and R₃ or R₁ and R₄ may form a cyclic structure (e.g., Formulas 4E and 4F).

Suitable analogs of acridine include

### Triarylmethane (compounds not according to the invention)

Triarylmethane or triarylmethane-type reductant is illustrated by a generalized structure (Formula 5). Referring to Formula 5, R₁, R₂, and R₃ are independently selected from the following group: H, alkyl moiety, aryl moiety, benzyl moiety, allyl moiety, amide moiety, ester moiety, ether moiety, hydroxyl moiety, amine moiety, any derivative thereof, and the like. In some embodiments, R₁, R₂, and R₃ may independently occupy more than one substitution position in their respective rings (e.g., Formula 5A and 5B).

Suitable analogs of triarylmethane include

### Triamine

Triamine or triamine-type reductant is illustrated by a generalized structure (Formula 6), wherein R₁, R₂, R₃, R₄, R₅, and R₆ are connected to form three cyclic rings (e.g., Formula 6A to 6C).

Z F Triamine compounds according to the invention are

### Aryl benzoimidazoline

Aryl benzoimidazoline or aryl benzoimidazoline-type reductant is illustrated by a generalized structure (Formula 7). Referring to Formula 7, X is N, O, or S. If X is N, R₁ and R₂ are each components independently selected from the following group: H, alkyl moiety, R₃ is selected from the following group: H, alkyl moiety, alkene moiety, alkyne moiety, aryl moiety, benzyl moiety, R₄ is selected from the following group: H, alkyl moiety, aryl moiety, benzyl moiety, allyl moiety, In some embodiments, R₄ may independently occupy more than one substitution position.

### Suitable analogs of aryl benzoimidaline includes

### Dioxolane

Dioxolane or dioxolane-type reductant is illustrated by a generalized structure (Formula 8). Referring to Formula 8, R is a component selected from the following group: H, alkyl moiety, allyl moiety, benzyl moiety, alkanol moiety,

### Suitable analogs of dioxolane include

### Diethercyclohexadiene (not according to the invention)

Diethercyclohexadiene or diethercyclohexadiene-type reductant is illustrated by a generalized structure (Formula 9). Referring to Formula 9, R is a component selected from the following group: H, alkyl moiety, allyl moiety, benzyl moiety, alkanol moiety, any derivative thereof, and the like.

### Suitable analogs of diethercyclohexadiene includes

### Cycloheptatriene (not according to the invention)

Cycloheptatriene or cycloheptatriene-type reductant is illustrated by a generalized structure (Formula 10). Referring to Formula 10, R is a component selected from the following group: H, alkyl moiety, allyl moiety, benzyl moiety, alkanol moiety, any derivative thereof, and the like. In some embodiments, R may occupy more than one substitution position (e.g., Formula 10B).

### Suitable analogs of cycloheptatriene includes

The hydride donors described herein may be synthesized or purchased from chemical vendors. The following examples are provided for illustrative purposes and are not intended to be limiting. DHPD and DHPD-type reductants can be synthesized via a scheme utilizing an off-on switchable acyl donor in the form of different 1,4 dihydropyridine amides (Org. Biomol. Chem. 2015, 13, 185-198). Dimethyl 3,5-dicarboxylatepyridine can be purchased from Sigma-Aldrich (St. Louis, MO) or prepared via known procedures (J. Am. Chem. Soc. 2000, 122, 9014-9018). Formula 6A can be synthesized by a known scheme (Syn. Comm. 1994, 24, 3109-3114). Paramethoxybenzene benzoimidazoline or para-tertbutylbenzene benzoimidazoline can be obtained adapting a known synthesis procedure (Syn. Comm. 1983, 13, 1033-1039). Formula 2F can be obtained by adapting a known synthesis procedure (Org. Lett. 2013, 75, 180-183).

### Fuel Compositions

The organic hydride-based donors of the present disclosure may be useful as additives in hydrocarbon fuels to prevent or reduce undesirable ignition events in combustion engines. When used in fuels, the proper concentration of the additive necessary in order to achieve the desired LSPI reduction or efficacy is dependent upon a variety of factors including the type of fuel used, the presence of other detergents or dispersants or other additives, etc. Generally, the range of concentration of the additives of the present disclosure in hydrocarbon fuel may range from 25 to 5000 parts per million (ppmw) by weight (including, but not limited to, 50 to 4000 ppm, 100 to 3500, 150 to 3000, 200 to 2500, 250 to 2000, 300 to 1500, 350 to 1000 and so forth). If other hydride donors are present in the fuel composition, a lesser amount of the additive may be used.

In some embodiments, the compounds of the present disclosure may be formulated as a concentrate using an inert stable oleophilic (i.e., soluble in hydrocarbon fuel) organic solvent boiling in a range of 65°C to 205°C. An aliphatic or an aromatic hydrocarbon solvent may be used, such as benzene, toluene, xylene, or higher-boiling aromatics or aromatic thinners. Aliphatic alcohols containing 2 to 8 carbon atoms, such as ethanol, isopropanol, methyl isobutyl carbinol, n-butanol and the like, in combination with the hydrocarbon solvents are also suitable for use with the present additives. In the concentrate, the amount of the additive may range from 10 to 70 wt. % (e.g., 20 to 40 wt. %).

In gasoline or gasoline fuels, other well-known additives can be employed including oxygenates (e.g., ethanol, methyl tert-butyl ether), other anti-knock agents, and detergents/dispersants (e.g., hydrocarbyl amines, hydrocarbyl poly(oxyalkylene) amines, succinimides, Mannich reaction products, aromatic esters of polyalkylphenoxyalkanols, or polyalkylphenoxyaminoalkanes). Additionally, friction modifiers, antioxidants, metal deactivators and demulsifiers may be present.

In diesel fuels, other well-known additives can be employed, such as pour point depressants, flow improvers, cetane improvers, lubricity additives and the like.

A fuel-soluble, non-volatile carrier fluid or oil may also be used with compounds of this disclosure. The carrier fluid is a chemically inert hydrocarbonsoluble liquid vehicle which substantially increases the non-volatile residue (NVR), or solvent-free liquid fraction of the fuel additive composition while not overwhelmingly contributing to octane requirement increase. The carrier fluid may be a natural or synthetic oil, such as mineral oil, refined petroleum oils, synthetic polyalkanes and alkenes, including hydrogenated and unhydrogenated polyalphaolefins, synthetic polyoxyalkylene-derived oils, such as those described in U.S. Patent Nos. 3,756,793; 4,191,537; and 5,004,478; and in European Patent Appl. Pub. Nos. 356,726 and 382,159.

The carrier fluids may be employed in amounts ranging from 35 to 5000 ppm by weight of the hydrocarbon fuel (e.g., 50 to 3000 ppm of the fuel). When employed in a fuel concentrate, carrier fluids may be present in amounts ranging from 20 to 60 wt. % (e.g., 30 to 50 wt. %).

### Lubricating Oil Compositions

The organic hydride-donors of the present disclosure may be useful as additives in lubricating oils to prevent or reduce undesirable ignition events in combustion engines. When employed in this manner, the additives are usually present in the lubricating oil composition in concentrations ranging from 0.001 to 10 wt. % (including, but not limited to, 0.01 to 5 wt. %, 0.2 to 4 wt. %, 0.5 to 3 wt. %, 1 to 2 wt. %, and so forth), based on the total weight of the lubricating oil composition. If other hydride donors are present in the lubricating oil composition, a lesser amount of the additive may be used.

Oils used as the base oil will be selected or blended depending on the desired end use and the additives in the finished oil to give the desired grade of engine oil, e.g. a lubricating oil composition having an Society of Automotive Engineers (SAE) Viscosity Grade of 0W, 0W-20, 0W-30, 0W-40, 0W-50, 0W-60, 5W, 5W-20, 5W-30, 5W-40, 5W-50, 5W-60, 10W, 10W-20, 10W-30, 10W-40, 10W-50, 15W, 15W-20, 15W-30, or 15W-40.

The oil of lubricating viscosity (sometimes referred to as "base stock" or "base oil") is the primary liquid constituent of a lubricant, into which additives and possibly other oils are blended, for example to produce a final lubricant (or lubricant composition). A base oil, which is useful for making concentrates as well as for making lubricating oil compositions therefrom, may be selected from natural (vegetable, animal or mineral) and synthetic lubricating oils and mixtures thereof.

Definitions for the base stocks and base oils in this disclosure are the same as those found in American Petroleum Institute (API) Publication 1509 Annex E ("API Base Oil Interchangeability Guidelines for Passenger Car Motor Oils and Diesel Engine Oils," December 2016). Group I base stocks contain less than 90% saturates and/or greater than 0.03% sulfur and have a viscosity index greater than or equal to 80 and less than 120 using the test methods specified in Table E-1. Group II base stocks contain greater than or equal to 90% saturates and less than or equal to 0.03% sulfur and have a viscosity index greater than or equal to 80 and less than 120 using the test methods specified in Table E-1. Group III base stocks contain greater than or equal to 90% saturates and less than or equal to 0.03% sulfur and have a viscosity index greater than or equal to 120 using the test methods specified in Table E-1. Group IV base stocks are polyalphaolefins (PAO). Group V base stocks include all other base stocks not included in Group I, II, III, or IV.

Natural oils include animal oils, vegetable oils (e.g., castor oil and lard oil), and mineral oils. Animal and vegetable oils possessing favorable thermal oxidative stability can be used. Of the natural oils, mineral oils are preferred. Mineral oils vary widely as to their crude source, for example, as to whether they are paraffinic, naphthenic, or mixed paraffinic-naphthenic. Oils derived from coal or shale are also useful. Natural oils vary also as to the method used for their production and purification, for example, their distillation range and whether they are straight run or cracked, hydrorefined, or solvent extracted.

Synthetic oils include hydrocarbon oil. Hydrocarbon oils include oils such as polymerized and interpolymerized olefins (e.g., polybutylenes, polypropylenes, propylene isobutylene copolymers, ethylene-olefin copolymers, and ethylenealphaolefin copolymers). Polyalphaolefin (PAO) oil base stocks are commonly used synthetic hydrocarbon oil. By way of example, PAOs derived from C₈ to C₁₄ olefins, e.g., C₈, C₁₀, C₁₂, C₁₄ olefins or mixtures thereof, may be utilized.

Other useful fluids for use as base oils include non-conventional or unconventional base stocks that have been processed, preferably catalytically, or synthesized to provide high performance characteristics.

Non-conventional or unconventional base stocks/base oils include one or more of a mixture of base stock(s) derived from one or more Gas-to-Liquids (GTL) materials, as well as isomerate/isodewaxate base stock(s) derived from natural wax or waxy feeds, mineral and or non-mineral oil waxy feed stocks such as slack waxes, natural waxes, and waxy stocks such as gas oils, waxy fuels hydrocracker bottoms, waxy raffinate, hydrocrackate, thermal crackates, or other mineral, mineral oil, or even nonpetroleum oil derived waxy materials such as waxy materials received from coal liquefaction or shale oil, and mixtures of such base stocks.

Base oils for use in the lubricating oil compositions of present disclosure are any of the variety of oils corresponding to API Group I, Group II, Group III, Group IV, and Group V oils, and mixtures thereof, preferably API Group II, Group III, Group IV, and Group V oils, and mixtures thereof, more preferably the Group III to Group V base oils due to their exceptional volatility, stability, viscometric and cleanliness features.

Typically, the base oil will have a kinematic viscosity at 100°C (ASTM D445) in a range of 2.5 to 20 mm²/s (e.g., 3 to 12 mm²/s, 4 to 10 mm²/s, or 4.5 to 8 mm²/s).

The present lubricating oil compositions may also contain conventional lubricant additives for imparting auxiliary functions to give a finished lubricating oil composition in which these additives are dispersed or dissolved. For example, the lubricating oil compositions can be blended with antioxidants, ashless dispersants, anti-wear agents, detergents such as metal detergents, rust inhibitors, dehazing agents, demulsifying agents, friction modifiers, metal deactivating agents, pour point depressants, viscosity modifiers, antifoaming agents, co-solvents, package compatibilizers, corrosion-inhibitors, dyes, extreme pressure agents and the like and mixtures thereof. A variety of the additives are known and commercially available. These additives, or their analogous compounds, can be employed for the preparation of the lubricating oil compositions of the invention by the usual blending procedures.

Each of the foregoing additives, when used, is used at a functionally effective amount to impart the desired properties to the lubricant. Thus, for example, if an additive is an ashless dispersant, a functionally effective amount of this ashless dispersant would be an amount sufficient to impart the desired dispersancy characteristics to the lubricant. Generally, the concentration of each of these additives, when used, may range, unless otherwise specified, from about 0.001 to about 20 wt. %, such as about 0.01 to about 10 wt. %.

### EXAMPLES

The following illustrative examples are intended to be non-limiting.

While LSPI can impact many types combustion engines, it can be particularly problematic in direct-injected, boosted (turbocharged or supercharged), spark-ignited (gasoline) internal combustion engines that, in operation, generate a brake mean effective pressure level of greater than 1000 kPa (10 bar) at engine speeds of from 1500 to 2500 rotations per minute (rpm), such as at engine speeds of from 1500 to 2000 rpm. Brake mean effective pressure (BMEP) is defined as the work accomplished during on engine cycle, divided by the engine swept volume, the engine torque normalized by engine displacement. The word "brake" denotes the actual torque or power available at the engine flywheel, as measured on a dynamometer. Thus, BMEP is a measure of the useful energy output of the engine.

It has now been found that the fuel compositions or lubricating oil compositions of this disclosure can prevent or minimize pre-ignition problems in internal combustion engines.

### EXAMPLES 1-8

The test compounds were blended in gasoline or lube oil and their capacity for reducing LSPI events were determined using the test method described below.

A General Motors (GM) 2.0L LHU 4-cylinder gasoline turbocharged direct-injected engine was used for LSPI testing. Each cylinder was equipped with a combustion pressure sensor.

A six-segment test procedure was used to determine the number of LSPI events that occurred under conditions of an engine speed of 2000 rpm and a load of 275 Nm. The LSPI test condition is run for 28 minutes with each segment separated by an idle period. Each segment is slightly truncated to eliminate the transient portion. Each truncated segment typically has approximately 110,000 combustion cycles (27,500 combustion cycles per cylinder). In total, the six truncated segments have approximately 660,000 combustion cycles (165,000 combustion cycles per cylinder).

LSPI-impacted combustion cycles were determined by monitoring peak cylinder pressure (PP) and crank angle at 5% total heat release (AI5). LSPI-impacted combustion cycles are defined as having both (1) a PP greater than five standard deviations than the average PP for a given cylinder and truncated segment and (2) an AI5 greater than five standard deviations less than the average for a given cylinder and truncated segment.

The LSPI frequency is reported as the number of LSPI-impacted combustion cycles per million combustion cycles and is calculated as follows: LSPI Frequency = [(Total Number of LSPI Impacted Combustion Cycles in Six Truncated Segments)/(Total Number of Combustion Cycles in Six Truncated Segments)] × 1,000,000

An additive associated with a test fuel and/or test lubricant that reduces the LSPI frequency, when compared to the corresponding baseline fuel and/or baseline lubricant, is considered an additive that mitigates LSPI frequency. For testing herein, the baseline fuel was a conventional 49-state premium unleaded gasoline fuel without any deposit control additives and the baseline lubricant was representative of a conventional engine oil meeting ILSAC GF-5 and API SN specifications. The test results are set forth in Table 1.

The examples summarize test results for various fuel or lubricating oil additives. For example, Example 1 shows result for DHPD as a fuel additive at 1000 ppmw in a test fuel fluid. The number of LSPI events observed when testing fuel or lubricant with additive is listed in column titled "LSPI Activity" while the number of LSPI events observed when testing fuel or lubricant without additive is listed in column titled "Reference." For a given example, inclusion or omission of the additives is the only difference between the fuel or lubricant compositions tested in the LSPI Activity and Reference columns.

**TABLE 1**

| | Additive Component (Formula #) | Additive Conc. | Base Fluid | LSPI Activity (events/million combustion cycles) | Reference (events/million combustion cycles) | Drop in LSPI Activity |
|---|---|---|---|---|---|---|
| Ex. 1 | DHPD (1A) | 1000 ppmw | Fuel | 41 | 254 | 84% |
| Ex. 2 | DHPD (1A) | 500 ppmw | Fuel | 30 | 358 | 92% |
| Ex. 3 | Triamine (6A) | 500 ppmw | Fuel | 179 | 239 | 25% |
| Ex. 4 | Triamine (6A) | 1000 ppmw | Oil | 322 | 461 | 30% |
| Ex. 5 | NADH analog (2F) | 500 ppmw | Fuel | 207 | 389 | 47% |
| Ex. 6 | NADH analog (2F) | 1000 ppmw | Oil | 78 | 220 | 64% |
| Ex. 7 | aryl benzoimidazoline (7A) | 1358 ppmw | Fuel | 28 | 319 | 91% |

## Claims

1. A fuel composition comprising (1) greater than 50 wt. % of a hydrocarbon fuel boiling in gasoline or diesel range and (2) a minor amount of one or more of organic hydride-based reductant, wherein the one or more organic hydride-based reductant is:
(a) a reductant as illustrated by Formulas 1A - 1K wherein Ar is an aryl moiety;
(b) a reductant as illustrated by Formulas 2A - 2F
(c) a reductant as illustrated by generalized structure Formula 3 wherein:
R₁, R₂, R₃, and R₄ are each independently selected from the following group: H, alkyl moiety, allyl moiety, and alkanol moiety; and
R₅ is selected from the following group: H, and alkyl moiety;
(d) a reductant as illustrated by generalized structure Formula 4 wherein X is N or O; and
when X is N:
R₁ is selected from the following group: H, alkyl moiety, allyl moiety, aryl moiety, and benzyl moiety;
R₂ is selected from the following group: H, alkyl moiety, allyl moiety, aryl moiety, benzyl moiety, and alkanol moiety;
R₃ and R₄ are each independently selected from the following group: H, alkyl moiety, aryl moiety, benzyl moiety, amine moiety, alkoxy moiety, and heteroatoms;
optionally wherein R₃ as well as R₄ independently occupy more than one substitution position within its respective rings; and
optionally wherein R₁ and R₃ or R₁ and R₄ form a cyclic structure;
when X is O, the reductant is as illustrated by structure Formula 4H
(e) a reductant as illustrated by Formulas 6A-6C
(f) a reductant as illustrated by generalized structure Formula 7 wherein:
X is N, O, or S;
when X is N:
R₁ and R₂ are each independently selected from the following group: H, and alkyl moiety;
R₃ is selected from the following group: H, alkyl moiety, alkene moiety, alkyne moiety, aryl moiety, and benzyl moiety; and
R₄ is selected from the following group: H, alkyl moiety, aryl moiety, benzyl moiety, and allyl moiety;
optionally wherein R₄ independently occupies more than one substitution position;
when X is O, the reductant is as illustrated by structure Formula 7I when X is S, the reductant is as illustrated by structure Formula 7J
(g) a reductant as illustrated by generalized structure Formula 8 wherein R is selected from the following group: H, alkyl moiety, allyl moiety, benzyl moiety, and alkanol moiety; or reductant as illustrated by structure Formulas 8D and 8E:

2. The fuel composition of claim 1, wherein the organic hydride-based reductant is present in 25 to 5000 ppm by weight.

3. The fuel composition of claim 1, wherein the organic hydride-based reductant is present in 250 to 2000 ppm by weight.

4. The fuel composition of claim 1, further comprising:
oxygenate, anti-knock agent, detergent, dispersant, friction modifier, antioxidant, metal deactivator, demulsifier, pour point depressant, flow improver, cetane improver, or lubricity additive.

5. Use of the fuel composition according to any one of claims 1-3 for preventing or reducing undesirable ignition events in an internal combustion engine, wherein the internal combustion engine is spark-ignited, operated at less than 3000 rpm, and operated under a load with a brake mean effective pressure of at least 1 MPa (10 bar).

6. Use of one or more organic hydride-based reductants as defined in claim 1 in a fuel composition to prevent or reduce low-speed pre-ignition events in an internal combustion engine, wherein the fuel composition is supplied to the engine and comprises greater than 50 wt. % of a hydrocarbon fuel boiling in gasoline range and a minor amount of the one or more of organic hydride-based reductants, and wherein the engine is spark-ignited, operated at less than 3000 rpm and operated under a load with a brake mean effective pressure of at least 1 MPa (10 bar).

7. A lubricating oil composition comprising (1) greater than 50 wt. % of a base oil and (2) a minor amount of one or more of an organic hydride-based reductant, wherein the one or more organic hydride-based reductant is:
(a) a reductant as illustrated by Formulas 1A - 1K wherein Ar is an aryl moiety;
(b) a reductant as illustrated by Formulas 2A - 2F
(c) a reductant as illustrated by generalized structure Formula 3 wherein:
R₁, R₂, R₃, and R₄ are each independently selected from the following group: H, alkyl moiety, allyl moiety, and alkanol moiety; and
R₅ is selected from the following group: H, and alkyl moiety;
(d) an reductant as illustrated by generalized structure Formula 4 wherein, X is N or O; and
when X is N:
R₁ is selected from the following group: H, alkyl moiety, allyl moiety, aryl moiety, and benzyl moiety;
R₂ is selected from the following group: H, alkyl moiety, allyl moiety, aryl moiety, benzyl moiety, and alkanol moiety;
R₃ and R₄ are each independently selected from the following group: H, alkyl moiety, aryl moiety, benzyl moiety, amine moiety, alkoxy moiety, and heteroatoms;
optionally wherein R₃ as well as R₄ independently occupy more than one substitution position within its respective rings; and
optionally wherein R₁ and R₃ or R₁ and R₄ form a cyclic structure;
when X is O, the reductant is as illustrated by structure Formula 4H
(e) a reductant as illustrated by Formulas 6A-6C wherein R₁, R₂, R₃, R₄, R₅, and R₆ are connected to form three cyclic rings;
(f) an reductant as illustrated by generalized structure Formula 7 wherein:
X is N, O, or S;
when X is N:
R₁ and R₂ are each independently selected from the following group: H, and alkyl moiety;
R₃ is selected from the following group: H, alkyl moiety, alkene moiety, alkyne moiety, aryl moiety, and benzyl moiety; and
R₄ is selected from the following group: H, alkyl moiety, aryl moiety, benzyl moiety, and allyl moiety;
optionally wherein R₄ independently occupies more than one substitution position;
when X is O, the reductant is as illustrated by structure Formula 7I
when X is S, the reductant is as illustrated by structure Formula 7J
(g) a reductant as illustrated by generalized structure Formula 8 wherein R is selected from the following group: H, alkyl moiety, allyl moiety, benzyl moiety, and alkanol moiety; or reductant as illustrated by structure Formulas 8D and 8E:

8. The lubricating oil composition of claim 7, wherein the organic hydride-based reductant is present in 0.001 to 10% by weight.

9. The lubricating oil composition of claim 7, wherein the organic hydride-based reductant is present in 0.5 to 5% by weight.

10. The lubricating oil composition of claim 7, further comprising:
antioxidant, ashless dispersant, anti-wear agent, detergent, rust inhibitor, dehazing agent, demulsifying agent, friction modifier, metal deactivating agent, pour point depressant, viscosity modifier, antifoaming agent, co-solvent, package compatibilizer, corrosion-inhibitor, dye, or extreme pressure agent.

11. Use of the lubricating oil composition according to any one of claims 7-10 for preventing or reducing undesirable ignition events in an internal combustion engine, wherein the internal combustion engine is spark-ignited, operated at less than 3000 rpm, and operated under a load with a brake mean effective pressure of at least 1 MPa (10 bar).

12. Use of one or more organic hydride-based reductants as defined in claim 7 in a lubricating oil composition to prevent or reduce low-speed pre-ignition events in an internal combustion engine, wherein the lubricating oil composition is supplied to the engine and comprises greater than 50 wt. % of a base oil and a minor amount of one or more of organic hydride-based reductant, and wherein the engine is spark-ignited, operated at less than 3000 rpm and operated under a load with a brake mean effective pressure of at least 1 MPa (10 bar).

## Patentansprüche

1. Kraftstoffzusammensetzung, umfassend (1) mehr als 50 Gew.-% eines im Benzin- oder Dieselbereich siedenden Kohlenwasserstoff-Kraftstoffs und (2) eine kleinere Menge eines oder mehrerer Reduktionsmittel auf Basis von organischem Hydrid, wobei es sich bei dem einen oder den mehreren Reduktionsmitteln auf Basis von organischem Hydrid um Folgendes handelt:
(a) ein Reduktionsmittel gemäß den Formeln 1A - 1K wobei Ar für eine Arylgruppierung steht;
(b) ein Reduktionsmittel gemäß den Formeln 2A - 2F
(c) ein Reduktionsmittel gemäß der verallgemeinerten Struktur der Formel 3 wobei:
R₁, R₂, R₃ und R₄ jeweils unabhängig aus der folgenden Gruppe ausgewählt sind: H, Alkylgruppierung, Allylgruppierung und Alkanolgruppierung; und
R₅ aus der folgenden Gruppe ausgewählt ist: H und Alkylgruppierung;
(d) ein Reduktionsmittel gemäß der verallgemeinerten Struktur der Formel 4 wobei X für N oder O steht; und
dann, wenn X für N steht:
R₁ aus der folgenden Gruppe ausgewählt ist: H, Alkylgruppierung, Allylgruppierung, Arylgruppierung und Benzylgruppierung;
R₂ aus der folgenden Gruppe ausgewählt ist: H, Alkylgruppierung, Allylgruppierung, Arylgruppierung, Benzylgruppierung und Alkanolgruppierung;
R₃ und R₄ jeweils unabhängig aus der folgenden Gruppe ausgewählt sind: H, Alkylgruppierung, Arylgruppierung, Benzylgruppierung, Amingruppierung, Alkoxygruppierung und Heteroatomen;
gegebenenfalls wobei R₃ sowie R₄ unabhängig mehr als eine Substitutionsposition in den jeweiligen Ringen besetzen; und
gegebenenfalls wobei R₁ und R₃ oder R₁ und R₄ eine cyclische Struktur bilden;
dann, wenn X für O steht, das Reduktionsmittel der Struktur der Formel 4H entspricht:
(e) ein Reduktionsmittel gemäß den Formeln 6A-6C ;
(f) ein Reduktionsmittel gemäß der verallgemeinerten Struktur der Formel 7 wobei:
X für N, O oder S steht;
dann, wenn X für N steht:
R₁ und R₂ jeweils unabhängig aus der folgenden Gruppe ausgewählt sind: H und Alkylgruppierung;
R₃ aus der folgenden Gruppe ausgewählt ist: H, Alkylgruppierung, Alkengruppierung, Alkingruppierung, Arylgruppierung und Benzylgruppierung; und
R₄ aus der folgenden Gruppe ausgewählt ist: H, Alkylgruppierung, Arylgruppierung, Benzylgruppierung und Allylgruppierung;
gegebenenfalls wobei R₄ unabhängig mehr als eine Substitutionsposition besetzt;
dann, wenn X für O steht, das Reduktionsmittel der Struktur der Formel 71 entspricht:
dann, wenn X für S steht, das Reduktionsmittel der Struktur der Formel 7J entspricht:
(g) ein Reduktionsmittel gemäß der verallgemeinerten Struktur der Formel 8 wobei R aus der folgenden Gruppe ausgewählt ist: H, Alkylgruppierung, Allylgruppierung, Benzylgruppierung und Alkanolgruppierung; oder Reduktionsmittel gemäß der Struktur der Formeln 8D und 8E:

2. Kraftstoffzusammensetzung nach Anspruch 1, wobei das Reduktionsmittel auf Basis von organischem Hydrid in einer Menge von 25 bis 5000 Gew.-ppm vorliegt.

3. Kraftstoffzusammensetzung nach Anspruch 1, wobei das Reduktionsmittel auf Basis von organischem Hydrid in einer Menge von 250 bis 2000 Gew.-ppm vorliegt.

4. Kraftstoffzusammensetzung nach Anspruch 1, ferner umfassend:
Oxygenat, Antiklopfmittel, Detergens, Dispergiermittel, Reibungsmodifikator, Antioxidans, Metalldesaktivator, Demulgator, Pourpoint-Erniedriger, Fließverbesserer, Cetanzahlverbesserer oder Schmieradditiv.

5. Verwendung der Kraftstoffzusammensetzung nach einem der Ansprüche 1-3 zur Verhinderung oder Verringerung von unerwünschten Zündereignissen in einem Verbrennungsmotor, wobei der Verbrennungsmotor fremdgezündet ist, bei weniger als 3000 U/min betrieben wird und unter einer Last mit einem mittleren Arbeitsdruck von mindestens 1 MPa (10 bar) betrieben wird.

6. Verwendung eines oder mehrerer Reduktionsmittel auf Basis von organischem Hydrid gemäß Anspruch 1 in einer Kraftstoffzusammensetzung zur Verhinderung oder Verringerung von Frühzündungsereignissen bei niedriger Drehzahl in einem Verbrennungsmotor, wobei die Kraftstoffzusammensetzung dem Motor zugeführt wird und mehr als 50 Gew.-% eines im Benzin- oder Dieselbereich siedenden Kohlenwasserstoff-Kraftstoffs
und eine kleinere Menge eines oder mehrerer Reduktionsmittel auf Basis von organischem Hydrid umfasst und wobei der Verbrennungsmotor fremdgezündet ist, bei weniger als 3000 U/min betrieben wird und unter einer Last mit einem mittleren Arbeitsdruck von mindestens 1 MPa (10 bar) betrieben wird.

7. Schmierölzusammensetzung, umfassend (1) mehr als 50 Gew.-% eines Grundöls
und (2) eine kleinere Menge eines oder mehrerer Reduktionsmittel auf Basis von organischem Hydrid, wobei es sich bei dem einen oder den mehreren Reduktionsmitteln auf Basis von organischem Hydrid um Folgendes handelt:
(a) ein Reduktionsmittel gemäß den Formeln 1A - 1K wobei Ar für eine Arylgruppierung steht;
(b) ein Reduktionsmittel gemäß den Formeln 2A - 2F ;
(c) ein Reduktionsmittel gemäß der verallgemeinerten Struktur der Formel 3 wobei:
R₁, R₂, R₃ und R₄ jeweils unabhängig aus der folgenden Gruppe ausgewählt sind: H, Alkylgruppierung, Allylgruppierung und Alkanolgruppierung; und
R₅ aus der folgenden Gruppe ausgewählt ist: H und Alkylgruppierung;
(d) ein Reduktionsmittel gemäß der verallgemeinerten Struktur der Formel 4 wobei X für N oder O steht; und
dann, wenn X für N steht:
R₁ aus der folgenden Gruppe ausgewählt ist: H, Alkylgruppierung, Allylgruppierung, Arylgruppierung und Benzylgruppierung;
R₂ aus der folgenden Gruppe ausgewählt ist: H, Alkylgruppierung, Allylgruppierung, Arylgruppierung, Benzylgruppierung und Alkanolgruppierung;
R₃ und R₄ jeweils unabhängig aus der folgenden Gruppe ausgewählt sind: H, Alkylgruppierung, Arylgruppierung, Benzylgruppierung, Amingruppierung, Alkoxygruppierung und Heteroatomen;
gegebenenfalls wobei R₃ sowie R₄ unabhängig mehr als eine Substitutionsposition in den jeweiligen Ringen besetzen; und
gegebenenfalls wobei R₁ und R₃ oder R₁ und R₄ eine cyclische Struktur bilden;
dann, wenn X für O steht, das Reduktionsmittel der Struktur der Formel 4H entspricht:
(e) ein Reduktionsmittel gemäß den Formeln 6A-6C wobei R₁, R₂, R₃, R₄, R₅ und R₆ unter Bildung von drei cyclischen Ringen verbunden sind;
(f) ein Reduktionsmittel gemäß der verallgemeinerten Struktur der Formel 7 wobei:
X für N, O oder S steht;
dann, wenn X für N steht:
R₁ und R₂ jeweils unabhängig aus der folgenden Gruppe ausgewählt sind: H und Alkylgruppierung;
R₃ aus der folgenden Gruppe ausgewählt ist: H, Alkylgruppierung, Alkengruppierung, Alkingruppierung, Arylgruppierung und Benzylgruppierung; und
R₄ aus der folgenden Gruppe ausgewählt ist: H, Alkylgruppierung, Arylgruppierung, Benzylgruppierung und Allylgruppierung;
gegebenenfalls wobei R₄ unabhängig mehr als eine Substitutionsposition besetzt;
dann, wenn X für O steht, das Reduktionsmittel der Struktur der Formel 7I entspricht:
dann, wenn X für S steht, das Reduktionsmittel der Struktur der Formel 7J entspricht:
(g) ein Reduktionsmittel gemäß der verallgemeinerten Struktur der Formel 8 wobei R aus der folgenden Gruppe ausgewählt ist: H, Alkylgruppierung, Allylgruppierung, Benzylgruppierung und Alkanolgruppierung; oder Reduktionsmittel gemäß der Struktur der Formeln 8D und 8E:

8. Schmierölzusammensetzung nach Anspruch 7, wobei das Reduktionsmittel auf Basis von organischem Hydrid in einer Menge von 0,001 bis 10 Gew.-% vorliegt.

9. Schmierölzusammensetzung nach Anspruch 7, wobei das Reduktionsmittel auf Basis von organischem Hydrid in einer Menge von 0,5 bis 5 Gew.-% vorliegt.

10. Schmierölzusammensetzung nach Anspruch 7, ferner umfassend:
Antioxidans, aschefreies Dispergiermittel, Verschleißschutzmittel, Detergents, Rostschutzmittel, Enttrübungsmittel, Demulgator, Reibungsmodifikator, Metalldesaktivierungsmittel,
Pourpoint-Erniedriger, Viskositätsmodifikator, Antischaummittel, Cosolvens, Paket-Kompatibilisator, Korrosionsschutzmittel, Farbstoff oder Höchstdruckadditiv.

11. Verwendung der Schmierölzusammensetzung nach einem der Ansprüche 7-10 zur Verhinderung oder Verringerung von unerwünschten Zündereignissen in einem Verbrennungsmotor, wobei der Verbrennungsmotor fremdgezündet ist, bei weniger als 3000 U/min betrieben wird und unter einer Last mit einem mittleren Arbeitsdruck von mindestens 1 MPa (10 bar) betrieben wird.

12. Verwendung eines oder mehrerer Reduktionsmittel auf Basis von organischem Hydrid gemäß Anspruch 7 in einer Schmierölzusammensetzung zur Verhinderung oder Verringerung von Frühzündungsereignissen bei niedriger Drehzahl in einem Verbrennungsmotor, wobei die Schmierölzusammensetzung dem Motor zugeführt wird und mehr als 50 Gew.-% eines Grundöls und eine kleinere Menge eines oder mehrerer Reduktionsmittel auf Basis von organischem Hydrid umfasst und wobei der Verbrennungsmotor fremdgezündet ist, bei weniger als 3000 U/min betrieben wird und unter einer Last mit einem mittleren Arbeitsdruck von mindestens 1 MPa (10 bar) betrieben wird.

## Revendications

1. Composition de combustible comprenant (1) plus de 50 % en poids d'un combustible hydrocarboné à point d'ébullition dans la plage de l'essence ou du diesel et (2) une quantité minoritaire d'un ou plusieurs agents réducteurs à base d'hydrure organiques, dans laquelle l'agent ou les agents réducteurs à base d'hydrure organiques sont :
(a) un agent réducteur tel qu'illustré par les formules 1A à 1K dans laquelle Ar est un groupement aryle ;
(b) un agent réducteur tel qu'illustré par les formules 2A à 2F
(c) un agent réducteur tel qu'illustré par la formule de structure généralisée 3 dans laquelle :
R₁, R₂, R₃ et R₄ sont choisis chacun indépendamment dans le groupe suivant : H, groupement alkyle, groupement allyle et groupement alcanol ; et
R₅ est choisi dans le groupe suivant : H, et un groupement alkyle ;
(d) un agent réducteur tel qu'illustré par la formule de structure généralisée 4 dans laquelle X est N ou O ; et
lorsque X est N :
R₁ est choisi dans le groupe suivant : H, groupement alkyle, groupement allyle, groupement aryle et groupement benzyle ;
R₂ est choisi dans le groupe suivant : H, groupement alkyle, groupement allyle, groupement aryle, groupement benzyle et alcanol ;
R₃ et R₄ sont choisis chacun indépendamment dans le groupe suivant : H, groupement alkyle, groupement aryle, groupement benzyle, groupement amine, groupement alcoxy et hétéroatomes ;
éventuellement dans laquelle R₃ ainsi que R₄ occupent indépendamment plus d'une position de substitution dans ses cycles respectifs ; et
éventuellement, dans laquelle R₁ et R₃ ou R₁ et R₄ forment une structure cyclique ;
lorsque X est O, l'agent réducteur est tel qu'illustré par la formule de structure 4H
(e) un agent réducteur tel qu'illustré par les formules 6A à 6C
(f) un agent réducteur tel qu'illustré par la formule de structure généralisée 7 dans laquelle :
X est N, O ou S ;
lorsque X est N :
R₁ et R₂ sont choisis chacun indépendamment dans le groupe suivant : H, et un groupement alkyle ;
R₃ est choisi dans le groupe suivant : H, groupement alkyle, groupement alcène, groupement alcyne, groupement aryle et groupement benzyle ; et
R₄ est choisi dans le groupe suivant : H, groupement alkyle, groupement aryle, groupement benzyle et groupement allyle ;
éventuellement, dans laquelle R₄ occupe indépendamment plus d'une position de substitution ;
lorsque X est O, l'agent réducteur est tel qu'illustré par la formule de structure 7I
lorsque X est S, l'agent réducteur est tel qu'illustré par la formule de structure 7J
(g) un agent réducteur tel qu'illustré par la formule de structure généralisée 8 dans laquelle R est choisi dans le groupe suivant : H, groupement alkyle, groupement allyle, groupement benzyle et groupement alcanol ; ou un agent réducteur comme illustré par les formules de structure 8D et 8E :

2. Composition de combustible selon la revendication 1, dans laquelle l'agent réducteur à base d'hydrure organique est présent en une quantité de 25 à 5 000 ppm en poids.

3. Composition de combustible selon la revendication 1, dans laquelle l'agent réducteur à base d'hydrure organique est présent en une quantité de 250 à 2000 ppm en poids.

4. Composition de combustible selon la revendication 1, comprenant en outre :
un composé oxygéné, un agent antidétonant, un détergent, un dispersant, un modificateur de friction, un antioxydant, un désactivateur de métaux, un désémulsifiant, un agent d'abaissement du point d'écoulement, un agent d'amélioration de l'écoulement, un agent d'amélioration de l'indice de cétane ou un additif de lubrification.

5. Utilisation de la composition de combustible selon l'une quelconque des revendications 1 à 3 pour empêcher ou réduire des événements d'allumage indésirables dans un moteur à combustion interne, dans laquelle le moteur à combustion interne est à allumage par étincelle, est exploité à moins de 3 000 tpm, et est exploité sous une charge avec une pression efficace moyenne de freinage d'au moins 1 MPa (10 bars).

6. Utilisation d'un ou plusieurs agents réducteurs à base d'hydrure organiques tels que définis dans la revendication 1 dans une composition de combustible pour empêcher ou réduire des événements de préallumage à basse vitesse dans un moteur à combustion interne, dans laquelle la composition de combustible est fournie au moteur et comprend plus de 50 % en poids d'un combustible hydrocarboné à point d'ébullition dans la plage de l'essence
et une quantité minoritaire d'un ou plusieurs agents réducteurs à base d'hydrure organiques, et dans laquelle le moteur est allumé par étincelle, est exploité à moins de 3 000 tpm et est exploité sous une charge avec une pression efficace moyenne de freinage d'au moins 1 MPa (10 bars).

7. Composition d'huile lubrifiante comprenant (1) plus de 50 % en poids d'une huile de base
et (2) une quantité minoritaire d'un ou de plusieurs agents réducteurs à base d'hydrure organiques, l'agent ou les agents réducteurs à base d'hydrure organiques étant :
(a) un agent réducteur tel qu'illustré par les formules 1A à 1K dans laquelle Ar est un groupement aryle ;
(b) un agent réducteur tel qu'illustré par les formules 2A à 2F
(c) un agent réducteur tel qu'illustré par la formule de structure généralisée 3 dans laquelle :
R₁, R₂, R₃ et R₄ sont choisis chacun indépendamment dans le groupe suivant : H, groupement alkyle, groupement allyle et groupement alcanol ; et
R₅ est choisi dans le groupe suivant : H, et un groupement alkyle ;
(d) un agent réducteur tel qu'illustré par la formule de structure généralisée 4 dans laquelle X est N ou O ; et
lorsque X est N :
R₁ est choisi dans le groupe suivant : H, groupement alkyle, groupement allyle, groupement aryle et groupement benzyle ;
R₂ est choisi dans le groupe suivant : H, groupement alkyle, groupement allyle, groupement aryle, groupement benzyle et alcanol ;
R₃ et R₄ sont choisis chacun indépendamment dans le groupe suivant : H, groupement alkyle, groupement aryle, groupement benzyle, groupement amine, groupement alcoxy et hétéroatomes ;
éventuellement dans laquelle R₃ ainsi que R₄ occupent indépendamment plus d'une position de substitution dans ses cycles respectifs ; et
éventuellement, dans laquelle R₁ et R₃ ou R₁ et R₄ forment une structure cyclique ;
lorsque X est O, l'agent réducteur est tel qu'illustré par la formule de structure 4H
(e) un agent réducteur tel qu'illustré par les formules 6A à 6C dans laquelle R₁, R₂, R₃, R₄, R₅ et R₆ sont reliés pour former trois cycles cycliques ;
(f) un agent réducteur tel qu'illustré par la formule de structure généralisée 7 dans laquelle :
X est N, O ou S ;
lorsque X est N :
R₁ et R₂ sont choisis chacun indépendamment dans le groupe suivant : H, et un groupement alkyle ;
R₃ est choisi dans le groupe suivant : H, groupement alkyle, groupement alcène, groupement alcyne, groupement aryle et groupement benzyle ; et
R₄ est choisi dans le groupe suivant : H, groupement alkyle, groupement aryle, groupement benzyle et groupement allyle ;
éventuellement, dans laquelle R₄ occupe indépendamment plus d'une position de substitution ;
lorsque X est O, l'agent réducteur est tel qu'illustré par la formule de structure 7I
lorsque X est S, l'agent réducteur est tel qu'illustré par la formule de structure 7J
(g) un agent réducteur tel qu'illustré par la formule de structure généralisée 8 dans laquelle R est choisi dans le groupe suivant : H, groupement alkyle, groupement allyle, groupement benzyle et groupement alcanol ; ou un agent réducteur comme illustré par les formules de structure 8D et 8E :

8. Composition d'huile lubrifiante selon la revendication 7, dans laquelle l'agent réducteur à base d'hydrure organique est présent en une quantité de 0,001 à 10 % en poids.

9. Composition d'huile lubrifiante selon la revendication 7, dans laquelle l'agent réducteur à base d'hydrure organique est présent en une quantité de 0,5 à 5 % en poids.

10. Composition d'huile lubrifiante selon la revendication 7, comprenant en outre :
un antioxydant, un dispersant sans cendres, un agent anti-usure, un détergent, un inhibiteur de rouille, un agent de débrumage, un agent de désémulsification, un modificateur de friction, un agent de désactivation de métaux, un agent d'abaissement du point d'écoulement,
un modificateur de viscosité, un agent antimousse, un co-solvant, un agent compatibilisant d'emballage, un inhibiteur de corrosion, un colorant ou un agent de pression extrême.

11. Utilisation de la composition d'huile lubrifiante selon l'une quelconque des revendications 7 à 10 pour empêcher ou réduire des événements d'allumage indésirables dans un moteur à combustion interne, dans laquelle le moteur à combustion interne est à allumage par étincelle, est exploité à moins de 3 000 tpm et est exploité sous une charge avec une pression efficace moyenne de freinage d'au moins 1 MPa (10 bars).

12. Utilisation d'un ou plusieurs agents réducteurs à base d'hydrure organiques tels que définis dans la revendication 7 dans une composition d'huile lubrifiante pour empêcher ou réduire les événements de préallumage à basse vitesse dans un moteur à combustion interne, dans laquelle la composition d'huile lubrifiante est fournie au moteur et comprend plus de 50 % en poids d'une huile de base et une quantité minoritaire d'un ou plusieurs agents réducteurs à base d'hydrure organiques, et dans laquelle le moteur est allumé par étincelle, est exploité à moins de 3 000 tpm et est exploité sous une charge avec une pression efficace moyenne de freinage d'au moins 1 MPa (10 bars).
